

## UNITED STATES PATENT OFFICE

2,594,547

FABRIC MATERIAL PROVIDED WITH  
PARAFFIN COATING

Karl A. Fischer, Washington, D. C.

No Drawing. Application May 14, 1948,  
Serial No. 27,100

4 Claims. (Cl. 117—168)

(Granted under the act of March 3, 1883, as  
amended April 30, 1928, 370 O. G. 757)

1

The invention described herein, if patented, may be manufactured and used by or for the Government for governmental purposes without the payment to me of any royalty thereon.

This invention relates to providing improved waterproofed and laundryproofed fabrics. More particularly, the invention is concerned with the application of synthetic paraffins having melting points over 100° C. to fabrics for improving their resistance to penetration by water and other non-solvent liquids or gases.

It has generally been attempted unsuccessfully to coat fabrics with paraffin or paraffin compositions which will retain some degree of permanency. Such coatings however, are found to be readily displaceable by laundry soaps or run at high washing temperatures, and therefore the practice has been to replenish the fabric with new coatings substantially after each washing. Further coatings, of a known character which may withstand high laundering temperatures, are in the nature of resins or modified resins which are not paraffins.

It is therefore an object of this invention to provide an improved paraffin coated fabric which will withstand high laundering temperatures.

It is another object of this invention to provide synthetic paraffin coatings on fabrics or the like as a surface coating or an impregnant to improve the fabric's resistance to climatic temperatures, water and laundering chemicals.

Further objects and advantages will be apparent from the following description.

It has been discovered that a synthetic paraffin in the nature of a neutral high melting point material secured from the hydrogenation of carbon monoxide has a melting point considerably above 100° C. and will adhere tenaciously to fabric materials considerably strengthening the threads or fibres giving them an improved shrinkproof characteristic. By placing a synthetic paraffin of this character, which melts at 120° C., in a suitable vat, heating it to approximately 130° C. or above its melting temperature, and thereafter immersing or dipping a fabric, in the nature of cloth or paper, into the melted paraffin, there will be deposited upon the surface of the fabric threads or fibres a coating of paraffin which congeals at temperatures over 100° C. Otherwise this paraffin may be applied by spraying in the melted condition or dissolved in a suitable solvent.

When such fabric is dipped or run through a paraffin vat, by suitable rollers or the like of conventional character, the molten synthetic paraffin penetrates into the weave or mesh of the fabric

adhering to the threads or fibre surfaces as a fine microcrystalline film of sufficient depth to provide a uniform coating thereover. A paraffin coating applied in this manner is relatively thin, being in the approximate nature of a few thousandths mm. thickness, which allows the fabric to retain its original flexibility and yet provides it with a stable coating resistant to high climatic temperatures and of a waterproof and laundryproof character. Fabrics treated with synthetic paraffins of this character are indifferent or neutral to acid and alkali reagents, such as used in laundering, and thereby provides the fabric, without further treatment, with a highly shrinkproof character. Further the fabrics are provided with a durable inexpensive coating which is easily applied without the use of extensive equipment or the need for expensive drying equipment.

In addition to the particular synthetic paraffin secured from by-products of the hydrogenation of carbon monoxide, as above indicated, it has also been found that other synthetic paraffins in the nature of those prepared by the Fischer-Tropsch synthesis, having melting points substantially from 100° C. to 150° C., will likewise produce impregnated, laminated and coated fabrics of improved waterproof and laundryproof characteristics. Further non-hydrolyzable plasticizers in the nature of polyvinyl ethers and esters or the like may be incorporated with these synthetic paraffins. Such mixtures may be, for example, a polyvinylbutyl ether and high melting point synthetic paraffin in the ratio of 1-3. The composition may be made by heating the ingredients to suitable melting temperatures or by dissolving them in a mutual organic solvent, as carbon tetrachloride or the like. Thereafter the fabric material may be dipped into or sprayed with the fluid composition to provide an improved coated fabric. It is apparent that the degree of saturation may be controlled by relative temperatures in melting. That is, at the approximate temperature of melting, or in the plastic stage, a heavier coating or saturation is secured by suitable roller or other impregnating means. Whereas, at higher temperatures a paraffin or paraffin mixture is thinner and provides a coating of the nature herein described. Likewise, fabric weave or fabric porosity will determine, in accordance with well known relative values to a great extent the penetration by paraffin materials of the character indicated.

With the paraffin, above indicated, a laminated fabric is produced by pressing two sheets of unshrunk cloth between rolls immersed in the

melted synthetic paraffin and thereafter the sheets when racked permit the paraffin to congeal at normal room temperature. This laminated sheet material does not separate under strenuous laundering conditions and no appreciable shrinkage occurs. Further, a lamination of two sheets of Troya tissue or a combination of cloth and paper materials, produced in the manner above described, withstands the heat and chemical conditions of laundering without separation and tissue when so treated is sufficiently strong to withstand comparatively rough handling through a series of fabricating operations.

With heavier paper and cloth material first impregnated with the molten synthetic paraffin described, in the manner as indicated, and then coated with a similar paraffin in a more plastic stage, an impervious sheeting is produced capable of being molded into containers and other desired forms which are capable of withstanding relatively high temperatures and are inert to non-solvent chemicals. For some purposes laminated structures of this character are preferred and may be produced by submersion and pressure as illustrated or the paraffin heated to substantially its melting point and applied in a plastic stage with conventional rollers.

From the above description it will be obvious that the improvements provided with the paraffin material set forth and other like synthetic paraffins or compositions in the nature as described may be utilized for analogous purposes substantially as illustrated and will come within the scope of the appended claims.

I claim:

1. A coated fabric carrying a fine microcrystalline film of a mixture of a synthetic paraffin obtained as a solid by-product in the hydrogenation of carbon monoxide according to the Fischer-Tropsch synthesis and of a member of the group consisting of polyvinyl ethers and polyvinyl esters as a plasticizer for said paraffin, said paraffin having a melting point in excess of 100° C., whereby said coated fabric is rendered capable of being laundered in boiling water.

2. A coated fabric carrying a fine microcrystal-

line film of a mixture of about 3 parts of a synthetic paraffin obtained as a solid by-product in the hydrogenation of carbon monoxide according to the Fischer-Tropsch synthesis and of about 1 part of a member of the group consisting of polyvinyl ethers and polyvinyl esters as a plasticizer for said paraffin, said paraffin having a melting point in excess of 100° C., whereby said coated fabric is rendered capable of being laundered in boiling water.

3. A coated fabric carrying a fine microcrystalline film of a mixture of a synthetic paraffin obtained as a solid by-product in the hydrogenation of carbon monoxide according to the Fischer-Tropsch synthesis and of polyvinyl butyl ether as a plasticizer for said paraffin, said paraffin having a melting point in excess of 100° C., whereby said coated fabric is rendered capable of being laundered in boiling water.

4. A coated fabric carrying a fine microcrystalline film of a mixture of about 3 parts of a synthetic paraffin obtained as a solid by-product in the hydrogenation of carbon monoxide according to the Fischer-Tropsch synthesis and of about 1 part polyvinyl butyl ether as a plasticizer for said paraffin, said paraffin having a melting point in excess of 100° C., whereby said coated fabric is rendered capable of being laundered in boiling water.

30 KARL A. FISCHER.

#### REFERENCES CITED

The following references are of record in the file of this patent:

#### 35 UNITED STATES PATENTS

| Number       | Name      | Date          |
|--------------|-----------|---------------|
| 2,149,329    | Ball      | Mar. 7, 1939  |
| 2,348,689    | Abrams    | May 9, 1944   |
| 40 2,352,328 | Kline     | June 27, 1944 |
| 2,373,634    | Wagner    | Apr. 10, 1945 |
| 2,443,221    | Bergstein | June 15, 1948 |

#### 45 OTHER REFERENCES

5 Scientific American, Jan. 25, 1945, page 29.